

1

3,745,039

## ELECTROLESS COBALT PLATING BATH AND PROCESS

Nathan Feldstein, Kendall Park, N.J., assignor to  
RCA Corporation

No Drawing. Continuation-in-part of application Ser. No. 872,750, Oct. 30, 1969. This application Oct. 28, 1971, Ser. No. 193,582

Int. Cl. C23c 3/02

U.S. Cl. 117—47 R

5 Claims 10

### ABSTRACT OF THE DISCLOSURE

Electroless deposition of cobalt from an aqueous alkaline bath on a palladium activated substrate. Bath contains hypophosphite as reducing agent, linear polyphosphate anion and ammonium hydroxide as complexing agents and small controlled amounts of nickel ion. Cobalt will also deposit without nickel ions being in bath by providing nickel strike on substrate.

This application is a continuation-in-part of application Ser. No. 872,750 filed Oct. 30, 1969 and now abandoned.

### BACKGROUND OF THE INVENTION

It has been well known that a number of metals may be deposited autocatalytically on various substrates, including some which are non-metallic, from a plating bath, without the use of an electric current. This type of process has become known as "electroless deposition." Some substrates require pre-treatment as with a catalyst, such as a palladium salt, prior to deposition of the metal. Other substrates themselves exert sufficient catalytic action without further preparatory treatment.

Cobalt is one of the metals which has been deposited by electroless techniques. One type of bath which has been used for electroless deposition of cobalt contains (a) a salt that furnishes cobalt ions, (b) a complexing agent for cobalt ions to prevent formation of undesired precipitates, (c) ammonium hydroxide which provides hydroxyl ions to maintain an alkaline pH and also aids in complexing the cobalt ions, and (d) a hypophosphite which serves as a reducing agent for the cobalt compounds. Other reducing agents such as amine boranes have also been tried in these baths.

Most of the baths that have previously been reported for electroless deposition of cobalt have operated at elevated temperatures (about 50° C.). At these temperatures it is difficult to maintain good control of the temperature and of the composition of the deposit.

Thin metallic films of cobalt or of cobalt-phosphorus alloys are of interest because of their magnetic properties. Some of the applications, such as high density recording systems in which these films may be used, require uniformity of magnetic properties. Cobalt films deposited by previously-known methods are not always satisfactory for such applications.

In comparison with films of other magnetic materials, such as nickel, cobalt deposits are harder and are more readily passivated.

### DESCRIPTION OF PREFERRED EMBODIMENT

In the baths of the present invention, complexing agents including linear polyphosphate anions contribute to obtaining improved cobalt films. A linear polyphosphate is a salt in which the phosphate anion has the formula  $(P_nO_{3n+1})^{-(n+2)}$ . An example of a preferred deposition bath is as follows.

2

### Example I

|                                                                   |        |     |
|-------------------------------------------------------------------|--------|-----|
| Na <sub>4</sub> P <sub>2</sub> O <sub>7</sub> .10H <sub>2</sub> O | g./l.  | 70  |
| CoSO <sub>4</sub> .7H <sub>2</sub> O                              | g./l.  | 50  |
| NH <sub>4</sub> OH conc. (approx. 58%)                            | cc./l. | 7.5 |
| (CH <sub>3</sub> ) <sub>2</sub> NHBH <sub>3</sub>                 | g./l.  | 1.5 |

In the above bath composition the amount of dimethylamine borane is based on room temperature operation. If the temperature is raised, the amount of borane can be decreased. Also, methylamine borane can be used as the reducing agent, and, since this substance is a stronger reducing agent than the corresponding dimethyl compound, smaller amounts are required. In general, the reducing agent in this example may be a substituted amine borane where the side chain is of low molecular weight such as methyl or ethyl. Other specific examples are monoethyl- and diethylamine borane. Tertiary butyl amine borane may also be used.

The preferred composition of Example I may be varied as follows:

|                                                                   |        |        |
|-------------------------------------------------------------------|--------|--------|
| CoSO <sub>4</sub> .7H <sub>2</sub> O                              | g./l.  | 7.6-50 |
| Na <sub>4</sub> P <sub>2</sub> O <sub>7</sub> .10H <sub>2</sub> O | g./l.  | 20-140 |
| NH <sub>4</sub> OH (approx. 58%)                                  | cc./l. | 2.3-30 |
| (CH <sub>3</sub> ) <sub>2</sub> NHBH <sub>3</sub>                 | g./l.  | 0.23-5 |

These baths operate at room temperature or above and yield cobalt-boron deposits on a wide variety of metals autocatalytically, including palladium-activated substrates. It has been found that cobalt-boron deposits of the present invention are self-initiating on substrates made of chromium, aluminum, molybdenum, tungsten, silver, copper and gold or any combination thereof.

Cobalt-boron deposits made with the baths of the present invention are also suitable for printed circuits and other similar applications. A pattern of the cobalt-boron is deposited on an activated, insulating substrate and a layer of copper or nickel is then deposited electrolytically on the cobalt-boron film.

Sodium hypophosphite may also be used as the reducing agent in the bath of the present invention. A preferred example using this type of reducing agent is as follows:

|                                                                   |        |     |
|-------------------------------------------------------------------|--------|-----|
| Na <sub>4</sub> P <sub>2</sub> O <sub>7</sub> .10H <sub>2</sub> O | g./l.  | 70  |
| CoSO <sub>4</sub> .7H <sub>2</sub> O                              | g./l.  | 50  |
| NH <sub>4</sub> OH conc. (approx. 58%)                            | cc./l. | 7.5 |
| Na <sub>2</sub> H <sub>2</sub> PO <sub>2</sub> H <sub>2</sub> O   | g./l.  | 26  |

This bath, like that of Example I, may be used at room temperature, although it has a slower plating rate. The plating rate may be increased by raising the temperature. The cobalt deposits as a cobalt-phosphorus alloy.

It has been found in accordance with the present invention that cobalt-phosphorus baths of the present system which includes a polyphosphate complexing agent, will not deposit spontaneously on insulating substrates (or other non-catalytic surfaces) even after these surfaces have been sensitized and activated in conventional manner with palladium. It has now been unexpectedly found, however, that if even small controlled amounts of nickel ion are present in the baths, the cobalt-phosphorus baths with polyphosphate complexing agent will deposit metal spontaneously on palladium-activated substrates. The cobalt-phosphorus will also deposit if a thin strike of nickel is first deposited on the substrate. By "thin strike" is meant at least about 500 Å. This is unexpected since, without nickel being present, the baths will not deposit on palladium which is a stronger catalyst than nickel.

The following is an example of carrying out this feature of the present invention. A glass surface is carefully cleaned, then sensitized by dipping in an aqueous sensitizing solution containing about 30 gms. of SnCl<sub>2</sub>·2H<sub>2</sub>O and 40 cc. concentrated hydrochloric acid per liter. After

thorough rinsing, the sensitized surface is activated by treating with an aqueous solution containing 1 gm. per liter of palladium chloride and 1 cc. per liter of concentrated hydrochloric acid. The sensitized and activated substrate is then utilized to deposit cobalt-phosphorus alloy as described below.

To test the effect of nickel on initiating cobalt deposition, bath were made up to be used at 20° C. and 40° C. as set forth below. The source of cobalt was  $\text{CoSO}_4 \cdot 7\text{H}_2\text{O}$  but it may be any soluble cobalt salt. Therefore, the cobalt is expressed in terms of  $\text{Co}^{++}$ .

|                                                                      | For use at<br>20° C. | For use at<br>40° C. |
|----------------------------------------------------------------------|----------------------|----------------------|
| $\text{Co}^{++}$ , g./l.                                             | 6                    | 6                    |
| $\text{Na}_4\text{P}_2\text{O}_7 \cdot 10\text{H}_2\text{O}$ , g./l. | 90                   | 90                   |
| $\text{NaH}_2\text{PO}_2 \cdot \text{H}_2\text{O}$ , g./l.           | 25                   | 25                   |
| $\text{NH}_4\text{OH}$ (58%), cc./l.                                 | 30                   | 105                  |

Using the above compositions, controlled additions of  $\text{NiSO}_4 \cdot 6\text{H}_2\text{O}$  were made with the following results. In the tables the nickel concentration is expressed as  $\text{Ni}^{++}$  since the nickel could be supplied by any soluble nickel salt.

TABLE I  
Results at 20° C. on Palladium-activated Substrate

|    | Concentration of added nickel as $\text{Ni}^{++}$ in g./l. | Approximate time to initiate plating (minutes) | Uniformity of plating |
|----|------------------------------------------------------------|------------------------------------------------|-----------------------|
| 1. | None                                                       | (1)                                            |                       |
| 2. | 0.223                                                      | 13                                             | Poor.                 |
| 3. | 0.446                                                      | 13                                             | Do.                   |
| 4. | 0.892                                                      | 4                                              | Acceptable.           |
| 5. | 1.34                                                       | 2                                              | Good.                 |
| 6. | 1.78                                                       | 2                                              | Do.                   |
| 7. | 2.23                                                       | 1.5                                            | Do.                   |

<sup>1</sup> No indication.

TABLE II  
Results at 40° C. on Palladium-activated Substrate

|    | Concentration of added nickel as $\text{Ni}^{++}$ in g./l. | Approximate time to initiate plating (minutes) | Uniformity of plating |
|----|------------------------------------------------------------|------------------------------------------------|-----------------------|
| 1. | None                                                       | >10                                            | Very poor.            |
| 2. | $1.12 \times 10^{-2}$                                      | 3                                              | Poor.                 |
| 3. | $2.76 \times 10^{-2}$                                      | 3                                              | Do.                   |
| 4. | $5.52 \times 10^{-2}$                                      | 0.5                                            | Good.                 |
| 5. | $11.2 \times 10^{-2}$                                      | 0.5                                            | Do.                   |

In order to further test the effects on self-initiation of a cobalt-phosphorus bath containing much smaller amounts of cobalt, the following bath was prepared.

|                                                              |        |      |
|--------------------------------------------------------------|--------|------|
| $\text{Co}^{++}$                                             | g./l.  | 1.6  |
| $\text{Na}_4\text{P}_2\text{O}_7 \cdot 10\text{H}_2\text{O}$ | g./l.  | 25.0 |
| $\text{NaH}_2\text{PO}_2 \cdot \text{H}_2\text{O}$           | g./l.  | 20.0 |
| $\text{NH}_4\text{OH}$ (58%)                                 | cc./l. | 8    |

This bath was tested by adding varying amounts of  $\text{NiSO}_4 \cdot 6\text{H}_2\text{O}$ .

TABLE III  
Results at 40° C. on Palladium-activated Substrate

|    | Concentration of added nickel as $\text{Ni}^{++}$ in g./l. | Approximate time to initiate plating (minutes) | Uniformity of plating |
|----|------------------------------------------------------------|------------------------------------------------|-----------------------|
| 1. | 0                                                          | (1)                                            |                       |
| 2. | 0.011                                                      | 8.0                                            | Poor.                 |
| 3. | 0.0275                                                     | 2.5                                            | Good.                 |
| 4. | 0.055                                                      | 2.5                                            | Do.                   |
| 5. | 0.110                                                      | 2.5                                            | Do.                   |
| 6. | 0.22                                                       | 2.5                                            | Do.                   |

<sup>1</sup> No plating after 10 minutes.

The various ingredients of these baths other than the nickel salt can be varied within the limits indicated in the previous examples in which no nickel compound was present. As the temperature of the bath rises, the amount of nickel needed to initiate good cobalt-phosphorus deposition decreases. However, even at room temperature, deposition can readily be initiated when the cobalt salt

concentration is relatively low, for example, like that of Table III above.

The cobalt can be obtained from soluble salts other than the sulfate and can be used in any amount up to saturation. As the cobalt concentration increases, the amount of nickel needed to initiate deposition decreases.

The composition of Example II may be varied as follows:

|    |                                                              |        |        |
|----|--------------------------------------------------------------|--------|--------|
| 10 | $\text{CoSO}_4 \cdot 7\text{H}_2\text{O}$                    | g./l.  | 7.6-50 |
|    | $\text{Na}_4\text{P}_2\text{O}_7 \cdot 10\text{H}_2\text{O}$ | g./l.  | 20-140 |
|    | $\text{NH}_4\text{OH}$ (approx. 58%)                         | cc./l. | 2.3-30 |
|    | $\text{NaH}_2\text{PO}_2 \cdot \text{H}_2\text{O}$           | g./l.  | 5-50   |

Sodium pyrophosphate is only one example of a compound containing a polyphosphate ion that can be used in the baths of the present invention. Another example is a tripolyphosphate ( $\text{P}_3\text{O}_{10}$ )<sup>-5</sup>.

Other metals such as nickel, iron, molybdenum and tungsten can be co-deposited with cobalt using the baths of the present invention, by incorporating ions such as  $\text{Ni}^{++}$ ,  $\text{Fe}^{++}$ ,  $\text{MoO}_4^{-2}$ , and  $\text{WO}_4^{-2}$ .

Although ammonium hydroxide has been given as an example of an agent which both aids in maintaining an alkaline pH and serves as a complexing agent, amines such as ethylene diamine can be substituted for the ammonium hydroxide.

I claim:

1. An aqueous plating bath for the electroless deposition of cobalt-phosphorus alloy comprising:

|    |                                                              |        |            |
|----|--------------------------------------------------------------|--------|------------|
| 30 | $\text{Co}^{++}$                                             | g./l.  | 1.6-10     |
|    | $\text{Na}_4\text{P}_2\text{O}_7 \cdot 10\text{H}_2\text{O}$ | g./l.  | 20-140     |
|    | $\text{NH}_4\text{OH}$ (58%)                                 | cc./l. | 2.3-105    |
|    | $\text{NaH}_2\text{PO}_2 \cdot \text{H}_2\text{O}$           | g./l.  | 5-50       |
| 35 | $\text{Ni}^{++}$                                             | g./l.  | 0.055-2.23 |

2. A method of depositing a cobalt-phosphorus alloy on a non-catalytic substrate comprising sensitizing said substrate and activating said substrate with palladium and then treating said activated substrate with a solution at about 20° C. comprising:

|                                                              |        |                  |
|--------------------------------------------------------------|--------|------------------|
| Co <sup>++</sup>                                             | g./l.  | 1.6-10           |
| $\text{Na}_4\text{P}_2\text{O}_7 \cdot 10\text{H}_2\text{O}$ | g./l.  | 20-140           |
| $\text{NH}_4\text{OH}$ (58%)                                 | cc./l. | 2.3-30           |
| $\text{NaH}_2\text{PO}_2 \cdot \text{H}_2\text{O}$           | g./l.  | 5-50             |
| $\text{Ni}^{++}$                                             | g./l.  | 0.892-about 2.23 |

3. A method of depositing a cobalt-phosphorus alloy on a non-catalytic substrate comprising sensitizing said substrate and activating said substrate with palladium and then treating said activated substrate with a solution comprising:

|                                                              |        |                        |
|--------------------------------------------------------------|--------|------------------------|
| Co <sup>++</sup>                                             | g./l.  | 1.6-10                 |
| $\text{Na}_4\text{P}_2\text{O}_7 \cdot 10\text{H}_2\text{O}$ | g./l.  | 20-140                 |
| $\text{NH}_4\text{OH}$ (58%)                                 | cc./l. | 2.3-30                 |
| $\text{NaH}_2\text{PO}_2 \cdot \text{H}_2\text{O}$           | g./l.  | 5-50                   |
| $\text{Ni}^{++}$                                             | g./l.  | About 0.055-about 0.22 |

60 4. A method of depositing a cobalt-phosphorus alloy on a non-catalytic substrate comprising sensitizing said substrate and activating said substrate with palladium and then treating said activated substrate with a solution comprising:

|                                                              |        |                      |
|--------------------------------------------------------------|--------|----------------------|
| Co <sup>++</sup>                                             | g./l.  | 1.6-10               |
| $\text{Na}_4\text{P}_2\text{O}_7 \cdot 10\text{H}_2\text{O}$ | g./l.  | 20-140               |
| $\text{NH}_4\text{OH}$ (58%)                                 | cc./l. | 2.3-105              |
| $\text{NaH}_2\text{PO}_2 \cdot \text{H}_2\text{O}$           | g./l.  | 5-50                 |
| $\text{Ni}^{++}$                                             | g./c.  | 0.0275 to about 2.23 |

65 5. A method of depositing a cobalt-phosphorus alloy on a non-catalytic substrate comprising sensitizing said substrate and activating said substrate with palladium, depositing a thin strike of nickel having a thickness of at least

about 500 Å. on said substrate, and then treating said substrate with a solution comprising:

Co<sup>++</sup> ----- g./l. 1.6-10  
 Na<sub>4</sub>P<sub>2</sub>O<sub>7</sub>·10H<sub>2</sub>O ----- g./l. 20-140  
 NH<sub>4</sub>OH (58%) ----- cc./l. 2.3-105  
 NaH<sub>2</sub>PO<sub>2</sub>·H<sub>2</sub>O ----- g./l. 5-50

|           |        |                     |             |
|-----------|--------|---------------------|-------------|
| 3,370,979 | 2/1968 | Schmeckenbecher     | 106-1 X     |
| 2,690,401 | 9/1954 | Gutzeit et al.      | 117-47 A    |
| 2,287,400 | 3/1958 | Eisenberg et al.    | 117-130 E   |
| 3,666,529 | 5/1972 | Wright et al.       | 117-50      |
| 3,024,134 | 3/1962 | Nixon et al.        | 117-130 E   |
| 3,597,267 | 8/1971 | Mallory, Jr. et al. | 106-1 X     |
| 3,607,389 | 9/1971 | Canegallo et al.    | 117-130 E X |

## References Cited

## UNITED STATES PATENTS

3,627,545 12/1971 Mallory, Jr. et al. ----- 117-130 E X  
 2,532,284 12/1950 Brenner et al. ----- 117-130 E X  
 3,423,214 1/1969 Koretzky ----- 106-1

ALFRED L. LEAVITT, Primary Examiner

10 J. R. BATTEEN, JR., Assistant Examiner

U.S. CL. X.R.

106-1; 117-50, 71 R, 130 E, 130 B, 160 R; 204-38 S